

## UNITED STATES PATENT OFFICE

2,034,563

## COPPER-SILICON-CADMIUM ALLOYS

Charles H. Davis, Cheshire, Elmer L. Munson, Naugatuck, and Cyril Stanley Smith, Cheshire, Conn., assignors to The American Brass Company, Waterbury, Conn., a corporation of Connecticut

No Drawing. Application April 26, 1935,  
Serial No. 18,368

13 Claims. (Cl. 75—1)

This invention relates to copper-silicon alloys and has for its principal object the improvement of the tensile strength and casting properties of such alloys by the addition of cadmium.

5 Although the copper-silicon alloys have been known for a long time, no commercial application of copper alloys containing more than very small quantities of silicon was made until the addition of manganese was found to render them more 10 workable (U. S. Patent No. 1,539,260—1925). Since that time the alloys have become of major industrial importance and a number of other 15 ternary or more complex alloys containing silicon have been developed. While in some cases the third or additional element is added for the purpose of improving the strength or corrosion resistance of the alloys, it is probable that in most cases the principal effect is in modifying the casting characteristics, for the binary copper-silicon 20 alloys are considered to be difficult to cast soundly and to be very liable to contain blowholes, shrinkage cavities and drossy inclusions.

In studying the effects of a number of elements on copper-silicon alloys we have found that the 25 addition of cadmium greatly improves the casting qualities of copper-silicon alloys. We believe this effect to be due partly to the effect of cadmium in dispelling and particularly in preventing the absorption of gases on account of its 30 own high vapor pressure at the usual temperatures of casting, and partly to the comparatively fusible character of the oxides or silicates formed on the surface of the metal when exposed to air. The oxide readily collects into drops and separates 35 from the alloy and is not liable to become easily entrained during casting as are the films or powdery particles formed when a pure copper-silicon is oxidized. Fortunately, the slag is not 40 so thin that it cannot readily be skimmed from

the surface of the metal when this is at the usual pouring temperature.

The amount of cadmium that we have found necessary to have the first beneficial effects is quite small, about 0.05 percent, but we have found that amounts even as high as 1.5 percent may be added before the malleability of the alloys commences to be seriously impaired, although beyond this point the alloys cannot be commercially hot or cold rolled. On account of the comparatively 10 high cost of cadmium it is also preferable not to use an excess of it, and for most purposes we prefer to use about 0.5 percent.

In Table I we have by way of example given the 15 tensile properties of some alloys representing our invention. These tests were made on strip 0.040 in. thick made by hot and cold rolling. The final reduction by cold rolling was 50 percent following 20 an annealing at a temperature of 700° C. The cadmium addition increases the strength and 25 hardness of the alloy without a large effect in the ductility, but the principal mechanical properties characteristic of the alloy come from the silicon content, which should be between 0.5 and 25 5.0 percent, depending on the strength and ductility required and will usually be greater than the cadmium content. For many general engineering purposes a silicon content of about 3 percent seems desirable, combined with a cadmium 30 content of about 0.5 percent, but it is obvious to anyone skilled in the art that higher amounts of silicon, up to about 5 percent, would be desirable if greater strength is required, and smaller amounts of silicon if severe forming operations 35 are to be encountered, or if for other reasons the alloy has to be unusually ductile. At the same time the cadmium content may be varied between the limits given above to maintain a suitable bal- 40

ance between the desired casting and fabricating qualities and cost.

have sometimes observed the presence of a thin film on the surface of the alloy after heat treat-

TABLE I  
Tensile properties of copper-silicon-cadmium alloys

| Alloy No. | Composition, percent |      | Hard (cold rolled)        |                                |                              |                                             | Soft (700° anneal)        |                                |                              |                                             |
|-----------|----------------------|------|---------------------------|--------------------------------|------------------------------|---------------------------------------------|---------------------------|--------------------------------|------------------------------|---------------------------------------------|
|           | Cd                   | Si   | Yield point, lbs./sq. in. | Tensile strength, lbs./sq. in. | Elongation in 2 in., percent | Rockwell hardness, B-100 kg. $\frac{1}{16}$ | Yield point, lbs./sq. in. | Tensile strength, lbs./sq. in. | Elongation in 2 in., percent | Rockwell hardness, B-100 kg. $\frac{1}{16}$ |
| 10        |                      |      |                           |                                |                              |                                             |                           |                                |                              |                                             |
| 2005      | 0.25                 | 2.91 | 62,700                    | 100,100                        | 6.8                          | 93.7                                        | 10,800                    | 52,000                         | 68.0                         | 29.0                                        |
| 2019      | 0.25                 | 2.85 | 64,450                    | 100,500                        | 4.5                          | 94.6                                        | 13,800                    | 54,300                         | 62.8                         | 36.4                                        |
| 2020      | 0.41                 | 2.79 | 63,900                    | 101,200                        | 6.5                          | 94.8                                        | 13,000                    | 53,300                         | 65.5                         | 33.4                                        |
| 2030      | 0.45                 | 3.03 | 67,400                    | 104,900                        | 5.0                          | 95.0                                        | 12,500                    | 54,300                         | 68.8                         | 35.5                                        |
| 2021      | 0.76                 | 2.87 | 66,850                    | 103,200                        | 5.5                          | 95.3                                        | 13,200                    | 53,400                         | 65.8                         | 33.8                                        |
| 2010      | 0.90                 | 2.90 | 65,800                    | 105,200                        | 6.5                          | 94.7                                        | 13,600                    | 54,400                         | 67.3                         | 38.0                                        |
| 2025      | 1.31                 | 2.98 | 68,000                    | 110,600                        | 5.8                          | 96.5                                        | 14,700                    | 55,700                         | 68.5                         | 41.8                                        |
| 2012      | 0.49                 | 1.89 | 65,200                    | 84,150                         | 6.8                          | 87.1                                        | 9,800                     | 40,200                         | 66.8                         | 7.4                                         |
| 2032      | 0.79                 | 2.26 | 66,100                    | 92,400                         | 7.3                          | 91.5                                        | 11,300                    | 46,000                         | 71.5                         | 16.8                                        |
| 2034      | 1.08                 | 1.98 | 68,200                    | 92,400                         | 5.8                          | 92.0                                        | 12,000                    | 44,100                         | 74.3                         | 16.8                                        |
| 2029      | 0.30                 | 0.93 | 60,200                    | 67,800                         | 3.3                          | 74.1                                        | 8,200                     | 36,200                         | 48.8                         | -8.4                                        |
| 20        | 0.81                 | 0.89 | 62,750                    | 72,500                         | 4.0                          | 79.3                                        | 8,000                     | 36,900                         | 49.8                         | -3.5                                        |
| 2033      | 1.19                 | 0.80 | 62,900                    | 71,800                         | 3.5                          | 79.4                                        | 9,100                     | 37,500                         | 52.5                         | -1.1                                        |
| 2023      | 0.78                 | 3.90 | 62,400                    | 115,000                        | 4.8                          | 98.2                                        | 20,800                    | 50,900                         | 26.5                         | 55.0                                        |
| 2022      | 0.93                 | 3.86 | 63,450                    | 117,700                        | 5.0                          | 98.8                                        | 23,000                    | 56,400                         | 33.3                         | 55.9                                        |
| 2026      | 1.03                 | 3.95 | 62,900                    | 118,100                        | 2.0                          | 99.3                                        | 22,000                    | 52,300                         | 28.8                         | 56.2                                        |
| 2024      | 0.73                 | 4.85 | 59,700                    | 111,300                        | 0.5                          | 99.7                                        | 29,000                    | 59,500                         | 21.0                         | 66.1                                        |
| 25        | 0.77                 | 1.43 | 65,400                    | 83,400                         | 4.0                          | 86.1                                        | 11,800                    | 40,500                         | 50.5                         | 12.7                                        |

Tests on strip 0.040 in. thick.

Hard alloys were cold rolled 50 percent reduction following annealing for one hour at 700° C. Soft alloys were annealed one hour at 700° C. after same rolling treatment.

The cadmium is added to the molten copper-silicon alloy preferably in the form of a copper-cadmium alloy containing 10 to 50 percent cadmium, since if it is added as pure cadmium the loss is very high due to the low boiling point of the element. It is an advantage to have some cadmium present in the charge to give the full benefit of its action during melting and for that reason a portion of scrap is always advisable. The silicon can be put in with the cold charge or it may be added (either as the element or as a copper-silicon alloy) to the molten metal, either before or after adding the cadmium.

The usual impurities may, of course, be present in the alloys.

In addition to their good casting qualities the alloys of copper, cadmium and silicon in the ranges given above will be found to be particularly desirable from the standpoint of fabrication. The alloys may be readily not rolled at suitable temperatures and can be extensively cold rolled. They lend themselves readily to the usual forming operations either in the hot or cold condition. No difficulty will be encountered in either soldering or brazing the alloys. The alloys may be welded by resistance, arc or flame methods and they are also particularly suited for use as a welding rod not only for welding material of similar composition but also other materials of different types both non-ferrous and ferrous.

They may be used in the form of castings, made in sand or chill molds or in forms fabricated from wrought sheet, rod or wire. They can be extruded, hot forged or hot pressed and in addition to the hot working they may be made into wires, rods, tubes, sheets and shapes, and also may be drawn, stamped or spun into cups and other forms of drawn metal articles. Certain of the alloys with low silicon may be used for electrical purposes, although the conductivity of the alloys is not very high.

The alloys are suitable for any application wherein their strength, ductility and corrosion resistance is of advantage. They take on a good polish and are of attractive color and appearance.

During the usual processes of fabrication we

ment, and we believe this to be definitely advantageous in increasing the resistance to corrosion under certain conditions.

The addition of cadmium materially improves the resistance of copper-silicon alloys to failure when exposed to stress in a steam atmosphere. As an example, an alloy of 3 percent silicon exposed to a certain load in a suitable steam atmosphere failed after 1 hour, while an alloy of 3 percent silicon, 1 per cent cadmium exposed under similar conditions of stress failed after 76½ hours. The alloys are therefore well suited for expansion joints, flexible pipe, diaphragms, valves, and other parts exposed to steam or hot water when under stress.

The alloys have high resistance to corrosion in the atmosphere and in both hot and cold, fresh and salt water. The alloys are also suited to the construction of parts of chemical plant exposed to dilute acid or other corrosive media for which copper alloys are not basically unsuited.

In cases where high machinability is desired, additions of small amounts of sulphur or lead may be made. When so used the sulphur content would be from 0.01 to approximately 0.5 percent, and the lead from approximately 0.05 to 1 percent.

We have found that the solid solubility of cadmium in copper-silicon alloys varies considerably with temperature and certain alloys are therefore susceptible to precipitation hardening by suitable heat treatment. For example, we have found that with 3 percent silicon the solubility limit is about 1.1 percent cadmium at 500° C. and 0.4 percent at 400° C.; with 2 percent silicon about 1.4 and 0.6 percent cadmium; and with 1 percent silicon about 1.8 and 0.7 percent cadmium at 500 and 400° C. respectively. The increase in strength and hardness obtainable after heat treatment is not large but may be useful in some applications. Precipitation is not accompanied by any appreciable loss of ductility and the alloys are not damaged by service at slightly elevated temperatures.

Having thus set forth the nature of our invention, what we claim is:

1. An alloy composed of approximately 0.5 to 5

- percent silicon, 0.05 to 1.5 percent cadmium, balance copper.
2. An alloy composed of approximately 3.0 percent silicon, 0.5 percent cadmium, balance copper.
3. An alloy composed of approximately 2.0 percent silicon, 0.5 percent cadmium, balance copper.
4. An alloy composed of approximately 1.0 percent silicon, 0.5 percent cadmium, balance copper.
5. The alloy according to claim 1 containing from 0.01 to 0.5 percent sulphur.
6. The alloy according to claim 1 containing from 0.05 to 1 percent lead.
7. The alloy according to claim 2 containing from 0.01 to 0.5 percent sulphur.
8. The alloy according to claim 2 containing from 0.05 to 1 percent lead.
9. An alloy composed of approximately 0.5 to 5 percent silicon, 0.05 to 1.5 percent cadmium, and balance copper; in which the silicon content exceeds the cadmium content.
10. A wrought metal article fabricated from an alloy composed of approximately 0.5 to 5 percent silicon, 0.05 to 1.5 percent cadmium, balance copper.
11. A wrought metal article fabricated from an alloy composed of approximately 3 percent silicon, 0.5 percent cadmium, and balance copper.
12. The wrought metal article of claim 9 containing 0.01 to 0.5 percent sulphur.
13. The wrought metal article of claim 10 containing from 0.05 to 1 percent lead.

CHARLES H. DAVIS.  
ELMER L. MUNSON.  
CYRIL STANLEY SMITH.